

## UNITED STATES PATENT OFFICE

1,992,752

## TAR COMPOSITION

William H. Kershaw, Forest Hills, N. Y., assignor  
to The Texas Company, New York, N. Y., a  
corporation of Delaware

No Drawing. Application July 31, 1931, Serial  
No. 554,372. In Canada July 22, 1930

8 Claims. (Cl. 106—32)

This invention relates to compositions of tar or of tar-like consistency, having characteristics and properties adapted to render them of superior value in their application to the purposes for which tars are employed, and is a continuation in part of my co-pending application, Serial No. 382,848, filed August 1, 1929, for Road tars and methods of making the same.

The invention contemplates an improved tar composition comprising a mixture of a tar derived from coal and a petroleum tar which is miscible therewith in all proportions. More specifically, the invention contemplates the preparation of mixtures of tars derived from coal or coal products, such as coal tar, coke oven tar, water gas tar, gas works tar and the like, with a petroleum tar obtained by the thermal conversion of mineral oils for the production of motor fuel.

The petroleum tar, or pitch, to which the invention has reference is obtained by cracking mineral oils for the production of gasoline as practiced, for example, in the coil type, the shell still type, the coil and still type, or the tube and tank type, of cracking process and wherein the oil is subjected to heat treatment in either the vapor or liquid phase under superatmospheric pressures, or at least at pressures substantially above atmospheric. Such operations produce only a relatively small percentage of gas, a large percentage of gasoline or motor fuel, and a considerable amount of heavy oil which is either cyclically distilled in this process or distilled in a separate operation to form a distillate charging stock and a tarry residue.

The heavy tar or pitch product resulting from this type of cracking operation, while sometimes referred to as cycle fuel tar, is quite generally known in the industry as pressure tar, and it will be hereinafter referred to as petroleum pressure tar.

This petroleum pressure tar is to be distinguished from the so-called petroleum residues resulting from the ordinary distillation of petroleum for the production of distillates of the kerosene or gas oil type and where only incipient or very slight cracking takes place, and the resulting residual material is practically like ordinary crude oil residue. It is also to be differentiated, on the other hand, from the tars produced by the very drastic cracking of gas oil for the manufacture of oil gas, which tars really fall almost directly into the coal tar class, being devoid of the many desirable characteristics

of pressure tar and, therefore, incapable of carrying into, or imparting to, a tar composition the advantages and desirable characteristics of the composition of my invention.

Heretofore, tar compositions for use in road construction, or as waterproofing, or surfacing materials, have been prepared which comprised mixtures of coal tar with small amounts of petroleum residue obtained from the ordinary distillation of crude petroleum, and which residues have been subjected to relatively very slight cracking only, as already mentioned. These mixtures have been unsatisfactory since such petroleum residues are not truly miscible with coal tars. On account of their wide divergence in character, it has been impossible to produce stable homogeneous compositions. At most, it is impossible to mix more than 20% or 25% of such petroleum residue with coal tars, and mixtures in which the petroleum content exceeded this amount have been entirely unsatisfactory.

Coal tars are useful in the trade on account of their quick-setting properties and rapid bonding qualities. On the other hand, coal tars, or tars derived from coal products, are very susceptible to changes in atmospheric temperature. They become quite soft at summer temperatures and quite brittle at winter temperatures, as a result of which paving and surfacing materials composed substantially entirely of coal tars or tars derived from coal are subject to rapid deterioration and failure in service.

In using tars of the coal tar type in the construction and maintenance of bituminous roadways, the quick-setting properties of these tars is of value. When ordinary petroleum residues derived from the simple distillation of crude petroleum are admixed with the tar, the quick-setting properties of the tar may be impaired to a greater or lesser extent. I have discovered, however, that petroleum pressure tars do not act like the ordinary petroleum residues and that such petroleum pressure tars may be admixed with coal tar to yield a product possessing the quick-setting and rapid bonding qualities of a straight coal tar product. Furthermore, the product thus obtained possesses a high degree of ductility and adhesiveness.

This petroleum pressure tar obtained by the cracking of mineral oils for the production of gasoline is completely miscible with coal tars or tars derived therefrom in all proportions and at moderate temperatures. Also, contrasted with coal tars, petroleum pressure tar is much less

susceptible to changes in atmospheric temperatures and does not exhibit the development of brittleness at low temperatures. It may be obtained having a very high degree of ductility as well as a high degree of adhesiveness, and I have found that, provided the melting point does not exceed about 140° F., petroleum pressure tar or pitch derived therefrom by distillation of the petroleum pressure tar to remove its lighter constituents has a much greater ductility than coal tar of the same melting point, for example, as follows:

| 15                  | Coal tar | Pressure tar |
|---------------------|----------|--------------|
| Melting point °F.   | 122      | 122          |
| Ductility at 77° F. | 75       | 200+         |

20 Above approximately 140° F. melting point, the ductility of the petroleum pressure tar may drop off rapidly and it is, therefore, advantageous to employ a petroleum pressure tar having a melting point not in excess of about 140° F. where a tar composition of very high ductility is desired.

25 Since petroleum pressure tar is miscible with coal tars in all proportions, it may, therefore, comprise from 75% to 85% of the composition and result in a product which retains not only the quick-setting and rapid bonding advantages of the coal tar but also has the greater stability and wearing qualities of the petroleum pressure tar, making the composition a better product than either of its ingredients and yet a product which 30 will meet all the specifications and uses to which coal tars have heretofore been put.

35 My improved composition is particularly well adapted for use as a road tar and, when properly prepared, is in all respects equal to and superior 40 to the road tars usually made in coal tar residuals and conforms to the specification requirements commonly in use. Its use, however, is not limited and it can be employed successfully as a pipe 45 coating, for waterproofing as a binder, in coal briquetting, in the manufacture of prepared roofing and roofing composed of alternate layers of saturated felt and bituminous material, and for other purposes where coal tars have been considered particularly desirable, and the following 50 description, which refers particularly to road tars, is only by way of illustrating one manner in which my invention may be employed and not as a limitation of my invention.

55 Among the general types of tars commonly used by road contractors are heavy binders, cold patches and surfacing materials; and these tars can be readily made according to my invention.

60 The heavy pitch or binder of my invention may also be used under certain State specifications as a base for the lighter grades of tar for cold and hot surfacing; and I have discovered that I can produce specification materials by thinning my 65 heavy binder to the proper consistency with the distillate from water gas tar or a coal tar, such as coke oven tar or gas works tar. In order to meet the distillation test of certain specifications, such as, for instance, the "cut back" product used for cold patch, it is necessary to redistil the water 70 gas tar distillate and to use a blend of the original distillate with a predetermined fraction. The re-distillation can, however, be avoided by utilizing a fractionating column in connection with the tar distilling apparatus and taking off sufficient dis-

tillate to form a residual product of the desired consistency.

In making the road tars of my invention, I first take a petroleum pressure tar and reduce it by distillation to a pitch of the proper consistency, unless it is already sufficiently reduced in the cracking process. I then mix with the pitch a tar such as water gas tar or coke oven tar, or the oils or pitches produced therefrom which are miscible with the pressure tar and the pitches produced therefrom, at moderate temperatures and in all proportions, forming perfectly homogeneous mixtures which possess the characteristic odor and appearance of tar and the high ductility and extreme stickiness common to liquid 15 and semi-liquid tar products.

The water gas tar or coke oven tar may or may not be reduced by distillation prior to mixing with the pitch made from the pressure tar, depending upon the characteristics of the materials themselves. The actual mixing of the pitch from pressure tar and water gas or coke oven tar can be carried out in any suitable manner. In these mixtures the petroleum pressure tar is generally the major component. In some instances I have 20 found it desirable to add to the aforesaid mixtures a relatively small percentage of a suitable distillate such as that produced during the distillation of water gas or coke oven tar. The analyses of the resulting mixtures conform fully 25 to the road tar specifications commonly used.

I have found that the heavy binder constitutes a suitable base for the production of lighter surfacing material or cold patch material when cut back with a distillate which may be obtained from the distillation of water gas or coke oven tars, the proportions of the two materials depending upon the characteristics of the materials themselves and the specifications to be met. It will be understood by those skilled in the art that, 30 owing to the inherent variability in the characteristics of tars in general, it is necessary to vary the proportions of all of the materials used and the procedure, therefore, requires continued laboratory control by analyses of the component materials and the final products.

35 It is obvious that pitches of various consistencies or tars of various consistencies can be used in carrying out my invention, but as illustrative of a particular method employed to meet a definite 40 requirement, I give the following example:

I take a petroleum pressure tar and reduce it by heat and steam to form a pitch of about 154° F. melting point and having a specific gravity at 77° F. of about 1.18, removing usually about 25% 45 of distillate. I then take a tar of relatively low viscosity of the type of water gas tar or coal tar, and reduce it by heat to a suitable consistency for fluxing the petroleum pressure tar, ordinarily 50 taking off about 25% of distillate. The reduced water gas tar has a specific gravity at 77° F. of about 1.095. The petroleum pressure tar and the reduced tar are then mixed in the proportion of 75% of the former and 25% of the latter, and this mixture is then cut back with a tar distillate, in 55 the proportion of 95% of the mixture and 5% of the tar distillate, which may conveniently be distillate from the water gas tar. The tar distillate has a specific gravity of about .920, an initial boiling point of 200° F. and an end point of about 60 450° F.

65 The mixture so produced constitutes a heavy binder, and its qualifications are shown in the following table in comparison with the specification limits of the New Jersey specification for 70 75

heavy binder (low carbon type), which specification is typical of those in common use:

|                                 | Specification limits (N. J.) | Product of the invention |
|---------------------------------|------------------------------|--------------------------|
| 5 Specific gravity at 77° F.    | 1.15 to 1.205.               | 1.151                    |
| Float test at 122° F.           | 80 to 110 seconds.           | 84                       |
| Insoluble in CS <sub>2</sub> .  | 5% maximum.                  |                          |
| 10 Distillation method D20-28T: |                              |                          |
| 0 to 33° F.                     | 1% maximum.                  | 0%                       |
| 0 to 45° F.                     | 3% maximum.                  | 3%                       |
| 0 to 51° F.                     | 11% maximum.                 | 7%                       |
| 0 to 57° F.                     | 22% maximum.                 | 13%                      |
| Melting point of residue.       | 149° F. maximum.             | 128° F.                  |

15 As further illustrative of an example of the production of a cold patch material, I take 82% of the binder produced in the manner described above and 18% of a mixture of two cuts of fractions from a column which is used on the still in the distillation of the water gas tar. These two cuts constitute about two-thirds of the total distillate from the tar. This mixture complies with the New Jersey Specification covering cold patch material, as shown in the following table:

|                                 | Specification limits (N. J.) | Product of the invention |
|---------------------------------|------------------------------|--------------------------|
| 30 Specific gravity at 77° F.   | 1.09 to 1.165.               | 1.110                    |
| Viscosity engler 104° F. 50cc.  | 407 to 517 seconds           | 471                      |
| Insoluble in CS <sub>2</sub> .  | 5% maximum.                  |                          |
| 35 Distillation Method D20-28T: |                              |                          |
| 0 to 33° F.                     | 3 to 10%.                    | 3%                       |
| 0 to 45° F.                     | 10 to 20%.                   | 14%                      |
| 0 to 51° F.                     | 18 to 30%.                   | 19%                      |
| 0 to 57° F.                     | 28 to 37%.                   | 24.5%                    |
| Melting point of residue.       | 140° F. maximum              | 138° F.                  |

40 A preferred embodiment of my invention has been illustrated and described for the purpose of showing one way in which the invention may be practiced, but the inventive idea upon which this application is based is broader than this illustrative embodiment thereof. For example, I have referred to certain tars such as water gas tar, coke oven tar and gas works tar, but my invention is not to be construed as being limited to the use of these tars only, and the tars mentioned specifically are merely illustrative of the class or type of materials contemplated by my invention. My invention is not, therefore, to be limited by this disclosure, reference being had to the appended claims for that purpose.

45 I claim:

50 1. An adhesive asphaltic tar composition having a high degree of ductility combined with quick-setting properties, comprising a mixture of a tar derived from a coal product and a petroleum pressure tar which is miscible therewith in all proportions to form mixtures which are stable in the absence of a stabilizing agent.

55 2. An adhesive tar composition forming a heavy road binder and having a high degree of ductility

combined with quick-setting properties, comprising a mixture of a gas works tar and a petroleum pressure tar which is miscible therewith in all proportions to form mixtures which are stable in the absence of a stabilizing agent.

60 3. An adhesive tar composition forming a heavy road binder and having a high degree of ductility combined with quick-setting properties, comprising a mixture of a gas works tar and a petroleum pressure tar having a melting point not in excess of 140° F. and miscible therewith in all proportions to form mixtures which are stable in the absence of a stabilizing agent.

65 4. An adhesive tar composition forming a heavy road binder and having a high degree of ductility combined with quick-setting properties, comprising a mixture of a coal tar and a petroleum pressure tar which is miscible therewith in all proportions, said mixture comprising a larger proportion of petroleum pressure tar than of said coal tar and forming a mixture which is stable in the absence of a stabilizing agent.

70 5. An adhesive tar composition forming a heavy road binder and having a high degree of ductility combined with quick-setting properties, comprising a mixture of a tar derived from a coal product and a petroleum pressure tar which has been reduced by distillation and which is miscible therewith in all proportions to form mixtures which are stable in the absence of a stabilizing agent.

75 6. An adhesive tar composition forming a heavy road binder and having a high degree of ductility combined with quick-setting properties, comprising a mixture of a residual tar formed by distilling tar derived from a coal product and a petroleum pressure tar which has been reduced by distillation, and which is miscible therewith in all proportions to form mixtures which are stable in the absence of a stabilizing agent.

80 7. A composition adapted for use in the construction and maintenance of bituminous roadways, comprising a heavy road binder formed as a mixture of a tar derived from a coal product and petroleum pressure tar which is miscible therewith in all proportions forming mixtures which are stable in the absence of a stabilizing agent, and softened or cut back with a distillate obtained in the distillation of the tar derived from coal.

85 8. A composition adapted for use in the construction and maintenance of bituminous roadways, comprising a heavy road binder formed as a mixture of a tar derived from a coal product and petroleum pressure tar which is miscible therewith in all proportions forming mixtures which are stable in the absence of a stabilizing agent, and softened or cut back with a distillate obtained in the distillation of gas works tar.

90 WILLIAM H. KERSHAW.